

2,928,777

## ELECTROLYTIC POLISHING OF METALS

George H. Smith, Blasdell, N.Y., assignor to Electro Process, Inc., Buffalo, N.Y.

No Drawing. Application December 16, 1950  
Serial No. 201,248

8 Claims. (Cl. 204—140.5)

The present invention relates to the electro-polishing of metals and has particular application to the polishing of iron, aluminum, magnesium, and copper and their alloys, such as high carbon steel, low carbon steel, mild alloy steel, cast iron, wrought iron, stainless steel, Monel, Inconel, and brass. The methods of electro-polishing herein disclosed are applicable to all types of shapes and forms as, for instance, plate, rods, "rigidized" metal, perforated metal, cold rolled and hot rolled steel and sheets, and the like, and the articles fabricated therefrom.

It is an important economic object of my invention to electro-polish metal objects in short periods of time and at low anode current densities on the order of 0.25 to 10 amperes per square inch.

It is an object of my invention to provide an improved method of polishing iron, aluminum and copper and alloys thereof, and a composition to be employed therefor.

It is a further object of my invention to provide a mirror-bright finish upon the surface of the metals with simultaneous deburring of the sharp edges.

It is a further object of the invention to provide metal products such as iron and its alloys which may be directly plated with copper, nickel, chrome or other plating metals usually employed in the art, without further preparation.

It is a further object of this invention to prepare a surface on such metals wherein there is a greater adherence of the plating metals to the metal base than has been possible heretofore by electro-polishing processes available.

It is well known to the art that a great number of methods have been proposed for the electro-polishing of steel and other metals. In general, the electrolyte was mainly composed of strong acids, such as sulfuric acid and/or ortho-phosphoric acid, or other acids such as hydrochloric, hydrofluoric, chromic and arsenic acids, nitric acid, etc., either used per se or when necessary in admixture in variable proportions with sulfuric acid.

To these inorganic acids, additions of a great variety of organic compounds were made which were supposed to provide considerable improvements over polishing solutions of a pure inorganic nature. These additives consisted mainly of aliphatic carboxylic acids, such as acetic acid, tartaric acid, citric acid and the like, as embodied in U.S. Patents, 2,335,354 and 2,331,721 to James N. Ostrofsky, and/or aliphatic alcohols, e.g. glycerol as disclosed in U.S. Patent 2,315,695 to Charles L. Faust, or sucrose or dextrose, or various substances known as inhibitors and buffers.

Some of these combinations have reached widespread application in the electrolytic polishing of stainless steels. However, the application of electrolytic polishing to steel and iron has not acquired any importance since the electrolytes proposed by the art have failed to meet the requirements for a mirror bright finish, deburring of the steel and the production of a surface that could be plated without further preparation.

The prior art further discloses the use of cresol sulfonic acid as an effective surface brightener as illustrated in

"Protective Treatment of Metals" by Harold Silman, published by Chapman & Hall, London, England, 1948, but extensive tests with the use of this additive failed to produce a mirror-bright finish of the steel surface. In fact, it hardly showed any improvement over the use of additives cited in the foregoing paragraphs, and does not seem to have ever been adopted on an industrial scale.

I have now found, in accordance with the present invention, that a very much superior polishing effect and a very smooth mirror-bright surface can be produced on iron, aluminum, magnesium and copper, and their alloys such as stainless steel, brass, Monel, Inconel and steel, more readily and at a lower cost than was heretofore possible; the employment of an electrolytic solution for electro-polishing consisting essentially of a mixture of (a) inorganic acids or a mixture of inorganic acids and aliphatic organic acids and (b) an aromatic sulfonic acid characterized by the following general formula:



in which Ar represents an aromatic radical, single, linked or condensed of the benzene, naphthalene, anthracene etc., series, and in which X is the integer 1, 2 or more.

According to my invention, lead, stainless steel or copper is used as the cathode for the direct current (which may be produced by means of a rectifier or a motor generator), the metal to be polished being the anode, both anode and cathode being substantially immersed in the electrolytic polishing solution.

It is an important object of my invention that the current densities employed are uniquely low as compared to the current densities advocated and used by the prior art and that I am able to polish iron and carbon steel with current densities as low as one-half to one ampere per square inch of anode surface, when the aromatic sulfonic acids of my invention are used in the electrolyte of the electro-polishing bath.

The electrolyte employed, according to my invention, is composed of a plurality of acids, one of which may be an aliphatic carboxylic acid, such as acetic or glycolic acid; the bath may include inorganic acids or mixtures thereof, such as phosphoric or sulfuric acid, or both, and an aromatic sulfonic acid of the general type described above. I have discovered that the addition to the electro-polishing electrolytes of an aromatic sulfonic acid or of a mixture of the aromatic sulfonic acids of this invention is indispensable if a mirror-bright finish on steel, stainless steel, aluminum, Monel, Inconel, magnesium, brass and copper, etc., is to be attained.

According to my invention I may use the aromatic sulfonic acid with phosphoric acid alone, if a bright polish is desired on brass, copper, aluminum, carbon and stainless steel, for instance; or, I may use the aromatic sulfonic acid with sulfuric acid to polish stainless steel, aluminum and carbon steel; or, I may use the aromatic sulfonic acid with both phosphoric and sulfuric acid to cause a bright mirror polish on aluminum, stainless steel, Monel, Inconel, magnesium, carbon steel and its alloys.

Small amounts of an aliphatic carboxylic acid of from 1% to 20% by weight of the electrolyte may also be used in the electro-polishing composition, according to the present invention, which additions broaden the scope of operating efficiency of such solutions over a wider range of temperatures. But, these additions are not essential to the achievement of a mirror-bright polish on any of the previously mentioned metals and alloys if the aromatic sulfonic acids are being used as illustrated by the examples given below.

Thus metals may be polished by immersing the metal to be treated as an anode in an electrolytic bath comprising 1 to 50% of an aromatic sulfonic acid of the type contemplated herein, and 50 to 90% by weight of 66%

Bé. sulfuric acid. Where an aliphatic carboxylic acid is employed in the bath the aliphatic carboxylic acid may be present from 1 to 70% by weight, the aromatic sulfonic acid from 1 to 50% by weight, with from 40 to 85% by weight of 66° Bé. sulfuric acid. It is possible to polish metals anodically in a bath of from 50 to 90% by weight of 66° Bé. sulfuric acid containing from 1 to 50% of benzene sulfonic acid.

The time of treatment may be varied over a wide range, depending upon the acid mixture used with the aromatic sulfonic acid and the quality of metal being polished. Under optimal conditions, stainless steel may be polished in one to two minutes; brass and copper in one to two minutes; aluminum, carbon steel, Monel, Inconel, magnesium, in two to four minutes.

The amounts of metal removed from the anode to be brightened are very minute; the amounts removed in two minutes with an electrode potential of 12 volts, and a typical electrolyte of the present invention is, for example, as follows:

|                        | Inches |
|------------------------|--------|
| Carbon steel           | 0.0015 |
| Aluminum               | 0.001  |
| Stainless steel (18-8) | 0.002  |
| Copper or brass        | 0.0025 |
| Monel and Inconel      | 0.002  |
| Magnesium              | 0.001  |

2-naphthol 3-6-8 tri-sulfonic acid have been found especially suitable for imparting a bright mirror finish to carbon steel, stainless steel, aluminum, Monel, Inconel and magnesium.

5 Concentrations of the aromatic hydrocarbon sulfonic acid, or mixtures thereof, of 1 to 20% by weight of the total weight of the electrolyte are effective in improving the lustre of these metals and alloys.

Especially suitable are mixtures of naphthylamine-10 sulfonic acids which are by-products and wastes from organic intermediates production, and contain sulfuric acid in high concentration and in particular, the mono, di and tri sulfonic acid derivatives of beta-naphthylamine when used as a mixture, as they occur in the waste liquor of beta-naphthylamine sulfonation.

15 The following examples are given as further illustrations of the several methods which I have found to give the desired results, but these examples should not be taken as a limitation of my invention but merely as illustrative thereof.

#### Example I

24.8% by weight of benzene sulfonic acid of a technical grade containing 71% free benzene mono-sulfonic acid, 37.4% by weight sulfuric acid 96%, 34.0% by weight ortho-phosphoric acid 85% and 3.8% by weight water.

| Metal                    | Time, Min. | Temp. of Bath | Cathode         | Volts | Amps. per Sq. In. | Nature of Finish           |
|--------------------------|------------|---------------|-----------------|-------|-------------------|----------------------------|
| Aluminum 2S 16H          | 3          | 80            | Copper          | 15    | 0.5               | Very bright smooth polish. |
| Stainless 18-8 17-chrome | 3          | 80            | do              | 10    | 2.3               | Very bright polish.        |
| Low carbon steel         | 5          | 70            | Lead            | 10    | 2.0               | Mirror-bright finish.      |
| High carbon steel        | 4          | 70            | do              | 8     | 1½                | Do.                        |
| Magnesium                | 1½         | 70            | Stainless steel | 8     | 1½                | Do.                        |

The aromatic sulfonic acids which may be used, according to this invention, are derived from aromatic hydrocarbons such as benzene, naphthalene, anthracene, acenaphthene, phenanthrene, retene (7-isopropyl-1-methyl-phenanthrene), fluorene, etc., and may contain one or more sulfonic acid radicals, usually not more than three, to induce solubility in the electrolyte. Aliphatic side chains may be present, such as methyl, isopropyl, butyl, etc., radicals. I have also found that, in many instances, the aromatic sulfonic acid may be substituted by an amino group or a nitro group, but that the presence of a hydroxyl group, in general, impairs the results to a considerable degree unless a plurality of sulfonic acid radicals is present.

Other substitutes, such as halogens, do not, in general, yield the desired results because of the too great insolubility generally inherent in the halogenated aromatic sulfonic acids.

Thus, the aromatic sulfonic acids which I usually prefer to use in the free acidic state, according to my invention, comprise the following examples:

- 60 Benzene mono sulfonic acid
- Benzene 1,3-di sulfonic acid
- Ortho-toluene mono sulfonic acid
- Para-toluene mono sulfonic acid
- Meta-toluene mono sulfonic acid
- Ortho-xylene-4 sulfonic acid
- 65 2,6 naphthalene di sulfo acid
- 2,7 naphthalene di sulfo acid
- Retene di sulfonic acid

The aromatic sulfonic acids of the benzene series, such as benzene-mono-sulfonic acid, I have found to be especially effective for polishing steel, stainless steel, aluminum and magnesium. The aromatic sulfonic acids of the naphthalene series especially the 2-naphthylamine 5-7 di-sulfonic acid, 2-naphthylamine 1-5-7 tri-sulfonic acid and

45 After the electro-polishing, the metals were rinsed in soft water or a solution of hard water containing 1% of a softening agent, such as ethylene diamine tetra acetic acid or a sequestrating agent for the calcium and magnesium salts present in the hard water, and dried. This procedure was generally followed in the accomplishment of all the examples given below:

#### Example II

50 Naphthalene 2,6 and 2,7 di-sulfonic acids in adequate quantities show excellent results on carbon steels, aluminum and stainless steel in the following electrolyte: 12.4% by weight 2,6 naphthalene di-sulfonic acid, 12.4% by weight 2,7 naphthalene di-sulfonic acid, 37.5% by weight sulfuric acid 96%, 34% by weight orthophosphoric acid 85% and 3.7% by weight water.

| Metal             | Time, Min. | Temp. of Bath | Cathode | Volts | Amps. per Sq. In. | Nature of Finish           |
|-------------------|------------|---------------|---------|-------|-------------------|----------------------------|
| Aluminum          | 3          | 75            | Lead    | 15    | 0.5               | Very bright smooth finish. |
| 18-8 stainless    | 2½         | 70            | do      | 10    | 2.0               | Very bright finish.        |
| 17 chrome         | 3          | 70            | do      | 12    | 2.5               | Do.                        |
| Low carbon steel  | 5          | 65            | do      | 8     | 1½                | Do.                        |
| High carbon steel | 4          | 65            | do      | 8     | 1½                | Do.                        |
| Magnesium         | 1½         | 65            | do      | 8     | 1½                | Mirror-bright finish.      |

#### Example III

18% by weight technical benzene sulfonic acid containing 90% free benzene mono-sulfonic acid, 4.5% sulfuric acid ( $H_2SO_4$ ), 1.8% bi-phenyl sulfone ( $C_6H_5)_2SO_2$  plus unaccounted for material consisting of water, benzol and unidentified organic byproducts, 38% by weight

sulfuric acid 96%, 40% by weight orthophosphoric acid 85% and 4% by weight water.

| Metal              | Time, Min. | Temp. of Bath | Cathode          | Volts | Amps. per Sq. In. | Nature of Finish            |
|--------------------|------------|---------------|------------------|-------|-------------------|-----------------------------|
| Aluminum, 28 1/2H. | 3          | 80            | Stainless steel. | 15    | 0.5               | Very bright, smooth finish. |
| Stainless 18-8.    | 3          | 80            | do               | 10    | 2.3               | Very bright polish.         |
| Low carbon steel.  | 5          | 70            | do               | 10    | 2.0               | Mirror-bright finish.       |
| High carbon Steel. | 4          | 70            | do               | 8     | 1/2               | Do.                         |
| Magnesium...       | 2          | 70            | do               | 8     | 1/2               | Do.                         |

*Example IV*

9.3% by weight of toluene sulfonic acid 80% para 20% ortho (94%) 45.8% by weight of 96%  $H_2SO_4$ , 38.5% by weight of 85% ortho-phosphoric acid, and 6.4% by weight of water.

| Metal                        | Time, Min. | Temp. of Bath | Cathode   | Volts | Amps. per Sq. In. | Nature of Finish           |
|------------------------------|------------|---------------|-----------|-------|-------------------|----------------------------|
| Aluminum alloy. <sup>1</sup> | 3          | 35            | Copper... | 10    | 0.5               | Smooth bright polish.      |
| Stainless 18-8.              | 2          | 35            | Lead...   | 10    | 2.3               | Very bright polish.        |
| Low carbon steel.            | 5          | 70            | do        | 10    | 1.0               | Very bright smooth polish. |

<sup>1</sup> 32 1/2H, i.e., 12.5% Si, 1.0 Mg, 0.9% Ni, 0.9% Cu, one-half hard.

*Example V*

The following electrolyte gives a mirror-bright polish on carbon steel and magnesium and consists of 4.8% by weight water, 7.8% by weight of technical glycolic acid, 40.2% by weight of sulfuric acid 96%, 38.4% by weight ortho-phosphoric acid 85%, and 8.8% by weight 71% benzene sulfonic acid. Very good results were obtained by using para-toluene sulfonic acid as a substitute for benzene sulfonic acid in this formula.

| Metal                     | Time, Min. | Temp. of Bath | Cathode          | Volts | Amps. per Sq. In. | Nature of Finish                   |
|---------------------------|------------|---------------|------------------|-------|-------------------|------------------------------------|
| Low carbon steel.         | 5          | 60            | Stainless steel. | 10    | 9.8               | Mirror-bright polish, good deburr. |
| Magnesium 18-8 stainless. | 2          | 60            | do               | 10    | 0.5               | Very bright polish.                |
| Aluminum...               | 2          | 60            | do               | 15    | 0.5               | Fair polish.                       |

*Example VI*

50% by weight para-toluene sulfonic acid (94%), 18.5% by weight benzene sulfonic acid (71%), 31.5% by weight orthophosphoric acid (85%).

| Metal             | Time, Min. | Temp. of Bath | Cathode | Volts | Amps. per Sq. In. | Nature of Finish    |
|-------------------|------------|---------------|---------|-------|-------------------|---------------------|
| Low carbon steel. | 5          | 60            | Lead... | 10    | 0.8               | Very bright polish. |

*Example VII*

The addition of aromatic sulfonic acids to orthophosphoric acids greatly improves the lustre and brightness of polish attained on copper and brass. Small quantities of para-nitrotoluene ortho-sulfonic acid or retene di-sulfonic acid are especially effective in improving the polish on brass and copper. An example of this electrolyte is: 79% by weight of 85% ortho-phosphoric acid,

5% by weight retene di-sulfonic acid and 16% by weight of water.

| Metal       | Time, Min. | Temp. of Bath | Cathode    | Volts | Amps. per Sq. In. | Nature of Finish      |
|-------------|------------|---------------|------------|-------|-------------------|-----------------------|
| Copper..... | 2          | 50            | Copper.... | 10    | 0.5               | Mirror-bright polish. |
| Brass.....  | 2          | 50            | do         | 10    | 0.5               | Do.                   |

Aromatic sulfonic acids in the field of electrolytic polishing are most effectively used in the percentages indicated in above examples, i.e., from 1 to 20% by weight of the bath.

However, smaller percentages may be used according to the case. Their effect on the final polish, the current consumption and time necessary to achieve a mirror-bright finish, is substantial. It is also possible, by varying the percentages of the aromatic sulfonic acids used, to obtain different shades on the polished surface which may vary from a brown tone on stainless steel, to the bluish brilliance of chrome plated steel.

Low carbon steel polished according to Example I gives a mirror-bright finish which can be plated with nickel or chrome without further preparation.

What is claimed is:

1. A method of anodically polishing metals which comprises immersing the metal to be treated for from 1 1/2 to 5 minutes as an anode in an aqueous electrolytic bath consisting of 1.0 to 50% by weight of an aromatic hydrocarbon sulfonic acid and 50 to 70% by weight of 85% orthophosphoric acid, the current being of sufficient density to overcome any etching and result in a polishing of the metal being used as an anode.

2. A method of anodically polishing metals which comprises immersing the metal to be treated for from 1 1/2 to 5 minutes as an anode in an electrolytic bath consisting of 1 to 50% by weight of an aromatic hydrocarbon sulfonic acid and a combination of inorganic acids of 40 to 90% by weight said inorganic acids being selected from the group consisting of sulfuric acid and orthophosphoric acid.

3. A method of anodically polishing metals which comprises immersing the metal to be treated for from 1 1/2 to 5 minutes as an anode in an electrolytic bath consisting of 1 to 50% by weight of an aromatic hydrocarbon sulfonic acid, 1 to 7% by weight of an aliphatic carboxylic acid and 40 to 90% by weight of a combination of phosphoric and sulfuric acid.

4. A method of anodically polishing metals which comprises immersing the metal to be treated for from 1 1/2 to 5 minutes as an anode in an electrolytic bath consisting of 1.0 to 50% by weight of benzene sulfonic acid and 50 to 79% by weight 85% ortho-phosphoric acid, the current being of sufficient density to overcome any etching and result in a polishing of the metal being used as an anode.

5. A method of anodically polishing metals which comprises immersing the metal to be treated for from 1 1/2 to 5 minutes as an anode in an electrolytic bath consisting of 1 to 7% of an aliphatic carboxylic acid, 1 to 50% by weight of sulfonic acid of the formula



where Ar is an aromatic hydrocarbon radical and n is an integer of less than 4 the remainder being substantially inorganic acid selected from the group of inorganic acids consisting of sulfuric acid and orthophosphoric acid.

6. A method of anodically polishing metals which comprises immersing the metal to be treated for from 1 1/2 to 5 minutes as an anode in an electrolytic bath consisting of 1 to 50% by weight of a sulfonic acid of the formula  $Ar(SO_2OH)_n$  where Ar is an aromatic hydrocarbon radical and n is an integer less than 4, and 40 to

90% by weight of a combination of phosphoric and sulfuric acids.

7. A method of anodically polishing metals which comprises immersing the metal to be treated for from 1½ to 5 minutes as an anode in an electrolytic bath consisting of 1 to 50% by weight of a sulfonic acid of the formula  $Ar(SO_2OH)_n$  where Ar is an aromatic hydrocarbon radical and n is an integer less than 4, and 1 to 7% by weight of an aliphatic carboxylic acid and 40 to 90% by weight of a combination of phosphoric and sulfuric acids.

8. A method of anodically polishing metals which comprises immersing the metal to be treated for from 1½ to 5 minutes as an anode in an electrolytic bath consisting of 1 to 50% benzene sulfonic acid in combination with 50 to 70% of inorganic acid selected from the group of inorganic acids consisting of sulfuric acid and orthophosphoric acid, the time, temperature and current densities of the bath being adjusted so as to achieve a bright polish.

5

10

20

## References Cited in the file of this patent

## UNITED STATES PATENTS

|           |                 |               |
|-----------|-----------------|---------------|
| 1,956,571 | Grillet         | May 1, 1934   |
| 2,335,354 | Ostrofsky       | Nov. 30, 1943 |
| 2,386,078 | Weisberg et al. | Oct. 2, 1945  |

## FOREIGN PATENTS

|         |               |               |
|---------|---------------|---------------|
| 504,026 | Great Britain | Apr. 17, 1939 |
| 594,932 | Great Britain | Nov. 21, 1947 |

## OTHER REFERENCES

"Richter's Organic Chemistry," vol. 2 (published in 1922), page 172.

15 "Chemical and Electroplated Finisher," by H. Silman, published in 1948 by Chapman and Hall, Ltd., pages 100, 101.